



US008431311B2

(12) **United States Patent**  
**Sugiura et al.**

(10) **Patent No.:** **US 8,431,311 B2**  
(45) **Date of Patent:** **Apr. 30, 2013**

(54) **RESIN-FILLED CARRIER FOR ELECTROPHOTOGRAPHIC DEVELOPER, AND ELECTROPHOTOGRAPHIC DEVELOPER USING THE RESIN-FILLED CARRIER**

(75) Inventors: **Takao Sugiura**, Kashiwa (JP); **Takeshi Gondo**, Kashiwasi (JP); **Hiromichi Kobayashi**, Naganeyama (JP)

(73) Assignee: **Powdertech Co., Ltd.**, Chiba (JP)

(\*) Notice: Subject to any disclaimer, the term of this patent is extended or adjusted under 35 U.S.C. 154(b) by 792 days.

(21) Appl. No.: **12/342,222**

(22) Filed: **Dec. 23, 2008**

(65) **Prior Publication Data**

US 2009/0176170 A1 Jul. 9, 2009

(30) **Foreign Application Priority Data**

Dec. 26, 2007 (JP) ..... 2007-334500  
Sep. 3, 2008 (JP) ..... 2008-226085

(51) **Int. Cl.**  
**G03G 9/00** (2006.01)

(52) **U.S. Cl.**  
USPC ..... **430/111.31**; 430/111.3; 430/111.4

(58) **Field of Classification Search** ..... 430/111.1,  
430/111.3, 111.31, 111.4

See application file for complete search history.

(56) **References Cited**

U.S. PATENT DOCUMENTS

5,427,884 A \* 6/1995 Ohtani et al. ..... 430/108.14  
5,998,076 A 12/1999 Mahabadi et al.  
6,528,225 B1 3/2003 Mahabadi et al.

2006/0194137 A1 \* 8/2006 Kobayashi et al. ..... 430/111.31  
2006/0269862 A1 \* 11/2006 Kobayashi et al. ..... 430/111.31  
2007/0048649 A1 3/2007 Kobayashi et al.  
2009/0263739 A1 \* 10/2009 Sugiura et al. ..... 430/111.32

FOREIGN PATENT DOCUMENTS

|    |               |         |
|----|---------------|---------|
| JP | 54-78137 A    | 6/1979  |
| JP | 5-40367 A     | 2/1993  |
| JP | 11-295933 A   | 10/1999 |
| JP | 11-295935 A   | 10/1999 |
| JP | 2006-337579 A | 12/2006 |
| JP | 2007-57943    | 3/2007  |
| JP | 2007-133100   | 5/2007  |
| JP | 2007-218955   | 8/2007  |

OTHER PUBLICATIONS

U.S. Appl. No. 12/033,384, filed Feb. 19, 2008, and entitled "Resin-Filled Ferrite Carrier for Electrophoto-Graphic Developer and Electrophotographic Developer Using the Ferrite Carrier".

U.S. Appl. No. 12/041,836, filed Mar. 4, 2008, and entitled "Resin-Filled Ferrite Carrier Forelectrophotographic Developer, Production Method thereof and Electrophotographic Developer Using the Ferrite Carrier".

U.S. Appl. No. 12/403,544, filed Mar. 13, 2009, and entitled "Resin-Filled Carrier for Electrophotographic Developer, and Electrophotographic Developer Using the Resin-Filled Carrier".

U.S. Appl. No. 12/342,222, filed Dec. 23, 2008, and entitled "Resin-Filled Carrier for Electrophotographic Developer, and Electrophotographic Developer Using the Resin-Filled Carrie".

\* cited by examiner

*Primary Examiner* — Stewart Fraser

(74) *Attorney, Agent, or Firm* — Greenblum & Bernstein, P.L.C.

(57) **ABSTRACT**

A resin-filled carrier for an electrophotographic developer obtained by filling resin into voids of a porous ferrite core material, wherein the porous ferrite core material has a pore volume of 0.055 to 0.16 mL/g and a peak pore size of 0.20 to 0.7  $\mu$ m, and an electrophotographic developer using this resin-filled carrier.

**15 Claims, No Drawings**

## 1

**RESIN-FILLED CARRIER FOR  
ELECTROPHOTOGRAPHIC DEVELOPER,  
AND ELECTROPHOTOGRAPHIC  
DEVELOPER USING THE RESIN-FILLED  
CARRIER**

BACKGROUND OF THE INVENTION

1. Field of the Invention

The present invention relates to a resin-filled carrier used in a two-component electrophotographic developer used in copiers, printers and the like. More specifically, the present invention relates to a resin-filled carrier for an electrophotographic developer having a high breakdown voltage and a high particle breaking strength, and an electrophotographic developer using this resin-filled carrier.

2. Description of the Related Art

Electrophotographic developing methods develop by adhering toner particles in a developer to an electrostatic latent image which is formed on a photoreceptor. The developer used in such methods can be classified as either being a two-component developer composed of toner particles and carrier particles, or a one-component developer which only uses toner particles.

Among such developers, as a developing method using a two-component developer composed of toner particles and carrier particles, a cascade method or the like has long been employed. However, currently magnetic brush methods using a magnet roll have become mainstream.

In a two-component developer, carrier particles act as a carrying substance for imparting the desired charge to the toner particles and transporting the toner particles thus-imparted with a charge to the surface of the photoreceptor to form a toner image on the photoreceptor by stirring the carrier particles with the toner particles in a developing box which is filled with the developer. Carrier particles remaining on the developing roll which supports the magnets return back into the developing box from this developing roll, and are then mixed and stirred with new toner particles for reuse over a certain time period.

Unlike one-component developers, in two-component developers the carrier particles are mixed and stirred with the toner particles to charge the toner particles. The carrier particles also have a transporting function and are easily controlled when designing the developer. Therefore, two-component developers are suitable for full color developing apparatuses in which high image quality is demanded and for apparatuses performing high-speed printing in which the reliability and durability of image sustainability are demanded.

In two-component developers which are used in such a manner, the image properties, such as image density, fogging, white spots, gradation and resolution, need to exhibit a certain value from the initial stage. Furthermore, these properties must not change during printing and have to be stably maintained. To stably maintain these properties, it is necessary for the properties of the carrier particles in the two-component developer to be stable.

Conventionally, various kinds of carrier, such as an iron powder carrier, a ferrite carrier, a resin-coated ferrite carrier, a magnetic powder-dispersed resin carrier and the like, have been used for the carrier particles forming a two-component developer.

In recent years the workplace has become more networked, evolving from an era of single-function copiers to multifunction devices. In addition, the type of service provided has shifted from a system in which a contracted repair worker carries out regular maintenance and replaces the developer

## 2

and other parts to a maintenance-free system. Further, demands from the market for even longer developer life are becoming much greater.

In view of these circumstances, Japanese Patent Laid-Open No. 5-40367 proposes many magnetic powder-dispersed carriers in which fine, magnetic microparticles are dispersed in a resin to extend developer life by making the carrier particles lighter.

Such a magnetic powder-dispersed carrier can reduce true density by reducing the amount of magnetic microparticles, thus reducing the stress from stirring. As a result, chipping or peeling of the coating can be prevented, whereby stable image properties for a long period of time can be obtained.

However, because a binder resin covers the magnetic microparticles, the magnetic powder-dispersed carrier has a high carrier resistance. Thus, there is the drawback that it is difficult to obtain sufficient image density.

In addition, since the magnetic microparticles are hardened by the binder resin, the magnetic powder-dispersed carrier has also had the drawbacks that the magnetic microparticles detach due to stirring stress or from shocks in the developing apparatus, and that the carrier particles themselves split, possibly as a result of having inferior mechanical strength as compared with the conventionally-used iron powder carrier or ferrite carrier. The detached magnetic microparticles or split carrier particles adhere to the photoreceptor, thereby becoming a factor in causing image defects.

Further, a magnetic powder-dispersed carrier has the drawback that since fine magnetic microparticles are used, remnant magnetization and coercive force increase, so that the fluidity of the developer deteriorates. Especially when a magnetic brush is formed on a magnet roll, the bristles of the magnetic brush stiffen due to the presence of remnant magnetization and coercive force, which makes it difficult to obtain high image quality. There is also the problem that even when the carrier leaves the magnet roll, because the carrier magnetic agglomerations do not come unloose and the carrier cannot be rapidly mixed with the supplied toner, the rise in the charge amount is poor, which causes image defects such as toner scattering and fogging.

In addition, while a magnetic powder-dispersed carrier can be produced by two methods, crushing or polymerization, the crushing method has a poor yield, and the polymerization method has a complicated production process. Thus, both methods have the problem of high costs.

A resin-filled carrier in which the voids in a porous carrier core material are filled with a resin has been proposed as a replacement for magnetic powder-dispersed carriers. For example, Japanese Patent Laid-Open No. 11-295933 and Japanese Patent Laid-Open No. 11-295935 disclose a carrier which comprises soft-magnetic cores or hard magnetic cores, a polymer contained in the pores of the cores, and a coating which covers the cores. These resin-filled carriers enable a carrier to be obtained having few shocks, a desired fluidity, a broad range of frictional charge values, a desired conductance and a volume average particle size that is within a certain range.

Japanese Patent Laid-Open No. 11-295933 discloses that various suitable porous solid core carrier substances, such as a known porous core, may be used as the core material. Japanese Patent Laid-Open No. 11-295933 states that it is especially important that the carrier is porous and has the desired fluidity, and that soft magnetism, porosity as represented by BET surface area and volume average particle size are properties which need to be given attention.

However, as is described in the examples of Japanese Patent Laid-Open No. 11-295933, for a porosity of about

1,600 cm<sup>2</sup>/g in BET surface area, a sufficient reduction in the specific gravity is not achieved even by filling with a resin, and thus such a carrier cannot cope with the recent ever increasing demands for lengthened developer life.

Japanese Patent Laid-Open No. 11-295933 also discloses that it is difficult to precisely control the specific gravity and mechanical strength of a carrier which has been filled with resin merely by controlling the porosity as represented by BET surface area.

The measurement principle of BET surface area is to measure the physical and chemical adsorption of a specific gas, which does not correlate with the porosity of the core material. In other words, it is typical for BET surface area to change depending on particle size, particle size distribution and nature of the surface material even for a core material that has hardly any pores. Thus, even if porosity is controlled using the BET surface area measured in the above-described manner, it cannot be said that the core material can be sufficiently filled with resin. If a large amount of resin is filled into a core material having a high BET surface area value but which is not porous, or into a core material which is not sufficiently porous, the resin which could not be filled remains by itself without closely adhering to the core material. In such a state, the left-over resin floats in the carrier, causing a large amount of agglomerates to form among the particles, whereby fluidity deteriorates. When agglomerates break apart during toner usage, charge properties fluctuate greatly, making it difficult to obtain stable properties.

Further, in Japanese Patent Laid-Open No. 11-295933, a porous core is used, and the total content of the resin filled in the cores and the resin which coats the surface of the cores is preferably about 0.5 to 10% by weight of the carrier. In the examples of Japanese Patent Laid-Open No. 11-295933, the greatest total content of the resins does not even reach 6% by weight of the carrier. With such a small amount of resin, the desired low specific gravity cannot be realized, meaning that a performance that is merely approximate to that of the conventionally used resin-coated carrier is obtained.

Japanese Patent Laid-Open No. 54-78137 discloses a carrier for an electrostatic image developer in which the pores and recesses on the surface of magnetic particles, which are either porous having a bulk specific gravity that is smaller than that of a substantially non-porous substance, or which have a large surface roughness, are filled with a fine powder consisting of an electrical insulating resin.

Japanese Patent Laid-Open No. 2006-337579 proposes a resin-filled carrier formed by filling a resin in a ferrite core material having a void fraction of 10 to 60%. Japanese Patent Laid-Open No. 2007-57943 proposes a resin-filled carrier which has a three-dimensional layered structure. Japanese Patent Laid-Open Nos. 2006-337579 and 2007-57943 disclose that various methods may be employed for filling the resin in the resin-filled carrier core material, such as a dry method, a spray-dry method using a fluidized bed, a rotary-dry method, and a liquid immersion-dry method using a universal stirrer, and that a suitable method is selected according to the core material and resin to be used.

Further, Japanese Patent Laid-Open No. 2007-57943 discloses that when filling the resin, since it is difficult to fill the voids with resin under an ordinary pressure or in a pressurized state, it is preferred to reduce the pressure inside the filling apparatus, so that the resin can be efficiently and sufficiently filled in the voids inside the particles, which makes it easier to form a three-dimensional layered structure.

Further, Japanese Patent Laid-Open No. 2007-133100 discloses a carrier in which a resin is impregnated in a porous magnetic body, and a carrier coated with a large amount of

resin on the surface of a core material. Since these carriers have a light true specific gravity, excess carrier can be smoothly discharged along with the toner by developing while supplying a supply developer having the toner and carrier to the developing apparatus, and as necessary using the carrier which is in excess in the developing apparatus interior in a two-component developing method supply developer which is discharged from the developing apparatus.

There are examples of the porous magnetic powder described in Japanese Patent Laid-Open Nos. 2006-337579, 2007-57943, 2007-133100 in which void volume of the core material is investigated by BET and oil absorption. However, BET only relates to surface area, and the actual level of voids cannot be found from the BET value. Further, while oil absorption does reflect void volume to a certain extent, considering oil absorption measurement principles, the gaps between the particles are also measured together with the voids in the particles, and thus oil absorption does not measure the actual void volume. Further, the gaps between the particles are usually larger than the actual void volume in the particles, so that oil absorption lacks accuracy as an index when trying to fill resin without any excess. Further, since Japanese Patent Laid-Open Nos. 2006-337579, 2007-57943, 2007-133100 do not describe the diameter of the voids which are present on the ferrite surface in which the resin is to be filled, or the distribution of such void diameters, when the resin is actually filled, there is filled resin unevenness among the particles and a lack of uniformity in resin filling. As a result, the particles which are not sufficiently filled with resin have poor strength, so that the carrier particles split and microparticles form during use in an actual machine, which are factors in image defects.

Japanese Patent Laid-Open No. 2007-218955 describes the pore size and pore volume of core material particles. Specifically, Japanese Patent Laid-Open No. 2007-218955 discloses that by providing, at the stage of the carrier core material prior to resin filling, durability capable of maintaining high resistance under high-voltage application conditions, maintenance of high-resistance during high-voltage application at the point when the carrier is used as an electro-photographic developer can be markedly improved, so that prevention of breakdown and prevention of a deterioration in image properties can be achieved. Further, Japanese Patent Laid-Open No. 2007-218955 discloses that for anti-spent properties as well, it is important to produce a porous magnetic powdered body having specific pore distribution properties, and to obtain a carrier core material by subjecting this porous magnetic powdered body to a treatment conferring high resistance.

However, it is known that in cases where both the pore distribution properties and the electrical resistance of the carrier core material are not satisfied, as in Comparative Example 4 of Japanese Patent Laid-Open No. 2007-218955, desired properties cannot be obtained.

This means that the pore distribution properties such as those described in Japanese Patent Laid-Open No. 2007-218955 are not sufficient. Thus, there is a need for a carrier core material which has more preferable pore distribution properties which are controlled more precisely.

In the above-described resin-filled carrier, there are the problems that charge tends to leak under a high voltage, breakdown voltage is low, the carrier particles may split or microparticles may be formed during strong stirring, and the particle breaking strength is low.

Thus, there is a need for a resin-filled carrier for an electro-photographic developer which, while maintaining the

advantages of the above-described resin-filled carriers, has a high breakdown voltage and a high particle breaking strength.

## SUMMARY OF THE INVENTION

Therefore, it is an object of the present invention to provide a resin-filled carrier for an electrophotographic developer which, while maintaining the advantages of the above-described resin-filled carriers, has a high breakdown voltage and a high particle breaking strength, and an electrophotographic developer using this resin-filled carrier.

As a result of extensive studies into resolving the above-described problems, the present inventors discovered that one of the causes of the problems that breakdown voltage and particle breaking strength are low is that there is an unevenness in filling degree among the particles, and that this unevenness can be resolved by setting the pore volume and the peak pore size of a porous ferrite core material within a specific range, thereby arriving at the present invention.

Specifically, the present invention provides a resin-filled carrier for an electrophotographic developer obtained by filling resin into voids of a porous ferrite core material, wherein the porous ferrite core material has a pore volume of 0.055 to 0.16 mL/g and a peak pore size of 0.20 to 0.7  $\mu\text{m}$ .

In the resin-filled carrier for an electrophotographic developer according to the present invention, in the pore size distribution of the porous ferrite core material, pore size unevenness  $dv$  represented by the following formula (I) is preferably 1.0 or less,

$$dv = |d_{84} - d_{16}|/2 \quad (1)$$

wherein  $d_{16}$  is a pore size calculated from the applied pressure on mercury when the mercury pressure penetration reaches 16%, where the total pressure penetration in the high pressure region is 100%; and  $d_{84}$  is a pore size calculated from the applied pressure on mercury when the mercury pressure penetration reaches 84%, in which the total pressure penetration in the high pressure region is 100%.

In the resin-filled carrier for an electrophotographic developer according to the present invention, the resin is filled in the porous ferrite core material preferably in an amount of 6 to 30 parts by weight based on 100 parts by weight of the porous ferrite core material.

The resin-filled carrier for an electrophotographic developer according to the present invention preferably has an average particle size of 20 to 60  $\mu\text{m}$ .

The resin-filled carrier for an electrophotographic developer according to the present invention preferably has a saturated magnetization of 30 to 80 Am<sup>2</sup>/kg.

The resin-filled carrier for an electrophotographic developer according to the present invention preferably has a pyconometer density of 2.5 to 4.5 g/cm<sup>3</sup>.

The resin-filled carrier for an electrophotographic developer according to the present invention preferably has an apparent density of 1.0 to 2.5 g/cm<sup>3</sup>.

Further, the present invention provides an electrophotographic developer composed of the above-described resin-filled carrier and a toner.

The electrophotographic developer according to the present invention may also be used as a supply developer.

Since the resin-filled carrier for an electrophotographic developer according to the present invention is a resin-filled ferrite carrier, and since weight can be reduced, durability is excellent, a longer life can be achieved, fluidity is excellent, and charge amount and the like can be easily controlled. Further, the inventive resin-filled carrier is stronger than a magnetic powder-dispersed carrier, and yet does not split,

deform or melt from heat or shocks. In addition, since the inventive resin-filled carrier has a specific pore size and pore volume, breakdown voltage is high, and particle breaking strength is also high.

## DETAILED DESCRIPTION OF THE PREFERRED EMBODIMENTS

Preferred embodiments for carrying out the present invention will now be described.

## &lt;Resin-Filled Carrier for an Electrophotographic Developer According to the Present Invention&gt;

The resin-filled carrier for an electrophotographic developer according to the present invention is obtained by filling a resin in the voids of a porous ferrite core material. This porous ferrite core material preferably includes at least one selected from the group consisting of Mn, Mg, Li, Ca, Sr, Cu and Zn. Considering the recent trend towards reducing environmental burden, such as restrictions on waste products, it is preferable for the heavy metals Cu, Zn and Ni to be contained in an amount which does not exceed the scope of unavoidable impurities (accompanying impurities).

This porous ferrite core material must have a pore volume of 0.055 to 0.16 mL/g, and a peak pore size of 0.2 to 0.7  $\mu\text{m}$ . Further, this porous ferrite core material preferably has a pore volume of 0.06 to 0.14 mL/g, and a peak pore size of 0.4 to 0.6  $\mu\text{m}$ .

If the pore volume of the porous ferrite core material is less than 0.055 mL/g, a reduction in weight cannot be achieved as a sufficient amount of resin cannot be filled. Further, if the pore volume is more than 0.16 mL/g, the carrier strength cannot be maintained even if the resin is filled.

If the peak pore size of the porous ferrite core material is less than 0.2  $\mu\text{m}$ , it becomes markedly more difficult to fill the resin as far as the core material center portion. Further, if the peak pore size is more than 0.7  $\mu\text{m}$ , the strength of the particles deteriorates due to the occurrence of extreme indents in the filled carrier. In addition, such a peak pore size is a factor in charge leakage and toner spent, and is thus not preferable.

Thus, resin-filled carrier with a suitably reduced weight can be obtained by setting the pore volume and the peak pore size in the above-described ranges, without the above-described various problems.

## (Pore Size and Pore Volume of the Porous Ferrite Core Material)

Measurement of the pore size and the pore volume of this porous ferrite core material may be carried out in the following manner. Specifically, measurement was carried out using the mercury porosimeters Pascal 140 and Pascal 240 (manufactured by Thermo Fisher Scientific). Using a CD3P (for powdered bodies) as a dilatometer, a sample was placed in a commercially-available capsule made from gelatin which had a plurality of opened holes, and this capsule was then placed in the dilatometer. After evacuating with the Pascal 140, mercury was filled therein. The low pressure region (0 to 400 kPa) was measured, and the results were taken as the first run. Next, evacuation and measurement of the low pressure region (0 to 400 kPa) were again carried out, and the results were taken as the second run. After the second run, the combined weight of the dilatometer, the mercury, the capsule, and the sample was measured. Next, the high pressure region (0.1 MPa to 200 MPa) was measured using the Pascal 240. Using the mercury pressure penetration obtained by the measurement of this high pressure portion, the pore volume, pore size distribution, and peak pore size of the porous ferrite core material were determined. Further, when determining the

pore size, the surface tension of the mercury was calculated as 480 dyn/cm and the contact angle as 141.3°.

In the resin-filled carrier for an electrophotographic developer according to the present invention, in the pore size distribution of the porous ferrite core material, the pore size unevenness dv is preferably 1.0 or less. Here, letting the total mercury pressure penetration in the high pressure region be 100%, the pore size calculated from the applied pressure on mercury when the mercury pressure penetration reaches 84% is given as  $d_{84}$ , and the pore size calculated from the applied pressure on mercury when the mercury pressure penetration reaches 16% is given as  $d_{16}$ . Further, the dv value was calculated from the following equation (1).

$$dv = |d_{84} - d_{16}|/2 \quad (1)$$

If the pore size unevenness dv of the porous ferrite core material is more than 1.0, there tends to be unevenness among the particles in their filled degree. Further, there also tends to be unevenness among the particles in their core material exposure degree after resin filling and unevenness within the individual particles. Such unevenness is a factor in the strength of the particles and the stability of the breakdown voltage being harmed. In addition, since indents on the surface of the particles become larger, such unevenness is a factor in charge leakage and toner spent.

The resin-filled carrier for an electrophotographic developer according to the present invention has a resin filled in a porous ferrite core material. The filled amount of resin is, based on 100 parts by weight of the porous ferrite core material, preferably 6 to 30 parts by weight, more preferably 6 to 20 parts by weight, and even more preferably 7 to 18 parts by weight, and most preferably 8 to 17 parts by weight. If the filled amount of resin is less than 6 parts by weight, a sufficient reduction in weight cannot be achieved, while if the filled amount of resin is more than 30 parts by weight, a large amount of remaining free resin which cannot all be filled is produced, which becomes a factor in problems such as charge defects and the like.

The resin to be filled is not especially limited, and may be appropriately selected according to the combined toner, the used environment and the like. Examples include a fluororesin, acrylic resin, epoxy resin, polyamide resin, polyamideimide resin, polyester resin, unsaturated polyester resin, urea resin, melamine resin, alkyd resin, phenol resin, fluoroacrylic resin, acryl-styrene resin, silicone resin, and a modified silicone resin modified by an acrylic resin, polyester resin, epoxy resin, polyamide resin, polyamideimide resin, alkyd resin, urethane resin, fluororesin or the like. Taking into consideration detachment of the resin due to mechanical stress during use, a thermosetting resin is preferably used. Specific examples of the thermosetting resin include an epoxy resin, phenol resin, silicone resin, unsaturated polyester resin, urea resin, melamine resin, alkyd resin, and a resin containing these.

A conductive agent may be added to the filled resin in order to control the electrical resistance of the carrier and the charge amount and charge speed. Since the electrical resistance of the conductive agent is itself low, there is a tendency for a charge leak to suddenly occur if the added amount is too large. Therefore, the added amount is 0.25 to 20.0% by weight, preferably 0.5 to 15.0% by weight and especially preferably 1.0 to 10.0% by weight, of the solid content of the filled resin. Examples of the conductive agent include conductive carbon, oxides such as titanium oxide and tin oxide, and various organic conductive agents.

In the filled resin, a charge control agent can be contained. Examples of the charge control agent include various charge

control agents generally used for toners and various silane coupling agents. This is because, although the charging capability is sometimes reduced if a large amount of resin is filled, it can be controlled by adding a charge control agent or a silane coupling agent. The charge control agents and coupling agents which may be used are not especially limited. Preferable examples of the charge control agent include a nigrosin dye, quaternary ammonium salt, organic metal complex and metal-containing monoazo dye. Preferable examples of the silane coupling agent include an aminosilane coupling agent and fluorinated silane coupling agent.

The resin-filled carrier for an electrophotographic developer according to the present invention is preferably surface-coated with a coating resin. Carrier properties, and especially electrical properties such as charge properties, are often affected by the materials present on the carrier surface and the shape of the carrier surface. Therefore, by coating the surface with a suitable resin, the desired carrier properties can be adjusted with good precision.

The coating resin is not especially limited. Examples include a fluororesin, acrylic resin, epoxy resin, polyamide resin, polyamideimide resin, polyester resin, unsaturated polyester resin, urea resin, melamine resin, alkyd resin, phenol resin, fluoroacrylic resin, acryl-styrene resin, silicone resin, and a modified silicone resin modified by an acrylic resin, polyester resin, epoxy resin, polyamide resin, polyamideimide resin, alkyd resin, urethane resin, fluororesin or the like. Taking into consideration detachment of the resin due to mechanical stress during use, a thermosetting resin is preferably used. Specific examples of the thermosetting resin include an epoxy resin, phenol resin, silicone resin, unsaturated polyester resin, urea resin, melamine resin, alkyd resin, and a resin containing these. The coated amount of the resin is preferably 0.5 to 5.0 parts by weight based on 100 parts by weight of the filled carrier (before resin coating).

A conductive agent and a charge control agent may be added to such coating resins for the same purpose as described above. The kind and added amount of the conductive agent and charge control agent are the same as for the case of the above-described filled resin.

The resin-filled carrier for an electrophotographic developer according to the present invention preferably has an average particle size of 20 to 60  $\mu\text{m}$ . Within this range, carrier adhesion can be prevented and good image quality can be obtained. If the average particle size is less than 20  $\mu\text{m}$ , this becomes a factor in carrier adhesion, and thus is not preferable. Further, if the average particle size is more than 60  $\mu\text{m}$ , this becomes a factor in image quality deterioration due to a deteriorating charging capability, and thus is not preferable. (Average Particle Size (Microtrac))

The average particle size was measured using a Microtrac Particle Size Analyzer (Model: 9320-X100), manufactured by Nikkiso Co., Ltd. Water was used for the dispersing solvent. A 100 mL beaker was charged with 10 g of a sample and 80 mL of water, and then 2 to 3 drops of a dispersant (sodium hexametaphosphate) were added therein. Next, using the ultrasonic homogenizer (Model: UH-150, manufactured by SMT Co. Ltd.), the output was set to level 4, and dispersing was carried out for 20 seconds. Then, the bubbles formed on the surface of the beaker were removed, and the sample was charged into the analyzer.

The resin-filled carrier for an electrophotographic developer according to the present invention preferably has a saturated magnetization of 30 to 80  $\text{Am}^2/\text{kg}$ . If the saturated magnetization is less than 30  $\text{Am}^2/\text{kg}$ , this is a factor in carrier adhesion, and thus is not preferable. If the saturated magne-

titization is more than 80 Am<sup>2</sup>/kg, the bristles of the magnetic brush stiffen, which makes it difficult to obtain good image quality.

(Saturated Magnetization)

Here, saturated magnetization may was measured using an integral-type B-H tracer BHU-60 (manufactured by Riken Densi Co., Ltd.). An H coil for measuring magnetic field and a 4 πI coil for measuring magnetization were placed in between electromagnets. In this case, the sample was put in the 4 πI coil. The outputs of the H coil and the 4 πI coil when the magnetic field H was changed by changing the current of the electromagnets were each integrated; and with the H output as the X-axis and the 4 πI coil output as the Y-axis, a hysteresis loop was drawn on recording paper. The measuring conditions were a sample filling quantity of about 1 g, the sample filling cell had an inner diameter of 7 mm±0.02 mm and a height of 10 mm±0.1 mm, and the 4 πI coil had a winding number of 30.

The pyconometer density of the resin-filled carrier for an electrophotographic developer according to the present invention is preferably 2.5 to 4.5 g/cm<sup>3</sup>. If the pyconometer density is less than 2.5 g/cm<sup>3</sup>, the carrier has too light a weight, so that charging capability tends to deteriorate. Further, if the pyconometer density is more than 4.5 g/cm<sup>3</sup>, the carrier weight reduction is insufficient, so that durability is poor.

(Pyconometer Density)

Pyconometer density was measured in the following manner. Specifically, measurement was carried out based on JIS R9301-2-1, using a pyconometer. Here, methanol was used as the solvent, and measurement was carried out at a temperature of 25° C.

The resin-filled carrier for an electrophotographic developer according to the present invention preferably has an apparent density of 1.0 to 2.5 g/cm<sup>3</sup>. If the apparent density is less than 1.0 g/cm<sup>3</sup>, the carrier has too light a weight, so that charging capability tends to deteriorate. Further, if the apparent density is more than 2.5 g/cm<sup>3</sup>, the carrier weight reduction is insufficient, so that durability is poor.

(Apparent Density)

The apparent density was measured according to JIS Z2504 (Apparent density test method for metal powders).

The resin-filled carrier for an electrophotographic developer of the present invention preferably has an electrical resistance for a 100 V applied voltage of 1×10<sup>7</sup>Ω or more. If the electrical resistance is less than 1×10<sup>7</sup>Ω, charge leakage and breakdown tend to occur during actual usage, and thus is not preferable.

(Electrical Resistance)

Non-magnetic parallel plate electrodes (10 mm×40 mm) are made to face each other with an inter-electrode interval of 1.0 mm. 200 mg of a sample is weighed and filled between the electrodes. The sample is held between the electrodes by attaching a magnet (surface magnetic flux density: 1500 Gauss, surface area in contact with the electrode: 10 mm×30 mm) to the parallel plate electrodes, and the resistance was measured by an insulation resistance tester (SM-8210, manufactured by DKK-TOA Corporation). The measurement was carried out in a constant temperature, constant humidity room controlled at a temperature of 25° C. and a humidity of 55%.

The resin-filled carrier for an electrophotographic developer of the present invention preferably has little unevenness among the particles in a filled state. If there is a lot of unevenness among the particles, this may cause a deterioration in breakdown voltage and particle breaking strength, and thus is not preferable. Further, it is preferred to have no splitting or microparticles. If splitting or microparticles are present, this

causes problems such as changing properties and white spots during use, and thus is not preferable.

(Unevenness Among Particles in the Filled Resin State)

5 The unevenness among the particles in the filled resin state was determined by observing the carrier at a magnification of 450 times with a scanning electron microscope (JSM-6100 model, manufactured by JEOL Ltd.).

10 The evaluation criteria for the unevenness among particles in the filled resin state are as follows.

Cases where no bias among the particles was observed in the filled degree of resin or exposure degree of the core material, and no agglomerated particles or free resin fine powder was observed, were evaluated with an “◎”. Cases where a slight bias among the particles was observed in the filled degree of resin or exposure degree of the core material, and a few agglomerated particles were observed, were evaluated with a “○”. Cases evaluated with an “◎” or a “○” were 15 considered to be in an acceptable range. Further, cases where a large bias among the particles was observed in the filled degree of resin or exposure degree of the core material, agglomerated particles or free resin fine powder was also observed, and a slight amount of resin which could not be 20 filled was observed on the carrier surface, were evaluated with a “Δ”. Cases where a marked bias among the particles was observed in the filled degree of resin or in the exposure degree of the core material, a large amount of agglomerated particles or free resin fine powder was also observed, and a large 25 amount of resin which could not be filled was observed on the carrier surface, were evaluated with a “X”. Cases evaluated with a “Δ” or a “X” were considered to be unacceptable.

(Carrier Strength Test (Evaluation Method of Splitting and Chipping, and Microparticles)

30 50 g of filled carrier was placed in a 50 cc glass bottle. This glass bottle was put into a cylindrical holder having a diameter of 130 mm and a height of 200 mm, set, and stirring was 35 then carried out for 360 minutes with a tumbler mixer.

40 After the stirring, the carrier was observed at a magnification of 450 times using a scanning electron microscope (JSM-6100 model, manufactured by JEOL Ltd.) to confirm the crushed state of the filled carrier. Carriers which had not changed after stirring were evaluated as an “◎”, and carriers for which a slight amount of chipping and microparticles, such as floating resin, produced by the crushing were 45 observed were evaluated with a “○”. Carriers evaluated with an “◎” or a “○” were considered to be in an acceptable range.

50 Carriers for which a large amount of chipping and microparticles, such as floating resin, were observed were evaluated with a “Δ”, and carriers for which a markedly large amount of chipping and microparticles, such as floating resin, were 55 observed were evaluated with a “X”. Carriers evaluated with a “Δ” or a “X” were considered to be unacceptable.

(Toner Spent)

60 The evaluation method for toner spent was as follows. Specifically, a developer having a toner concentration of 7% was prepared. The prepared developer was stirred for 36 hours, and then the carrier only was stripped from the developer. The spent toner was rinsed with toluene, and then the transmittance (%) of light having a wavelength of 560 nm of the resultant supernatant was measured using a visible light 65 spectrophotometer (MODEL 6100, manufactured by Jenway). A transmittance of 95% or more was evaluated as acceptable.

## 11

<Method for Producing the Resin-Filled Carrier for an Electrophotographic Developer According to the Present Invention>

The method for producing the resin-filled carrier for an electrophotographic developer according to the present invention will now be described.

In the method for producing the resin-filled carrier for an electrophotographic developer according to the present invention, to produce the porous ferrite core material, first, the raw materials are appropriately weighed, and then the resultant mixture is crushed and mixed by a ball mill, vibration mill or the like for 0.5 hours or more, and preferably for 1 to 20 hours. Although the raw materials are not especially limited, it is preferred to select the raw materials so that a composition is formed containing the above-described elements.

The resultant crushed matter is pelletized using a pressure molding machine or the like, and calcined at a temperature of 700 to 1,200° C. This may also be carried out without using a pressure molding machine, by after the crushing adding water to form a slurry, and then granulating using a spray drier. The calcined matter is further crushed by a ball mill, vibration mill or the like, and then charged with water, and optionally with a dispersant, a binder or the like to adjust viscosity. The resultant solution is then granulated by a spray drier. In the case of crushing after calcination, the calcined matter may be charged with water and crushed by a wet ball mill, wet vibration mill or the like.

The above crushing machine such as the ball mill or vibration mill is not especially limited, but, for uniformly and effectively dispersing the raw materials, preferably uses fine beads having a particle size of 1 mm or less as the media to be used. By adjusting the size, composition and crushing time of the used beads, the crushing degree can be controlled.

Then, sintering is carried out at a temperature of 800 to 1,500° C. in an atmosphere having a controlled oxygen concentration while holding the obtained granulated matter for 1 to 24 hours. At this stage, a rotary electric furnace, a batch-type electric furnace, a continuous electric furnace or the like may be used. The oxygen concentration of the atmosphere during the sintering may be controlled by pumping in an inert gas such as nitrogen, or a reducing gas such as hydrogen or carbon monoxide. Further, if using a rotary electric furnace, the sintering may be carried out multiple times while changing the atmosphere and sintering temperature.

The resultant sintered matter is crushed and classified. The particles are adjusted to a desired size using a conventionally-known classification method, such as air classification, mesh filtration and precipitation.

Thereafter, the electrical resistance can be optionally adjusted by heating the surface at a low temperature to carry out an oxide film treatment. The oxide film treatment may be conducted using a common furnace such as a rotary electric furnace or batch-type electric furnace, and the heat-treatment may be carried out, for example, at 300 to 700° C. The thickness of the oxide film formed by this treatment is preferably 0.1 nm to 5 µm. If the thickness is less than 0.1 nm, the effect of the oxide film layer is small, and thus is not preferable. If the thickness is more than 5 µm, the magnetization may decrease and the resistance may become too high, which makes it difficult to obtain the desired properties, and thus is not preferable. Reduction may optionally be carried out before the oxide film treatment. In this manner, a porous ferrite core material is prepared having a pore volume and a peak pore size in a specific range.

The pore volume, peak pore size, and pore size unevenness of the ferrite core material of such a carrier for an electrophotographic developer may be controlled in various ways, for

## 12

example according to the kind of raw material to be blended, the crushing degree of the raw materials, whether calcination is carried out, the calcination temperature, the calcination time, the binder amount during granulation by a spray drier, the sintering method, the sintering temperature, the sintering time, reduction by hydrogen or carbon monoxide gas and the like. These control methods are not especially limited. One such example will now be described below.

Specifically, pore volume tends to increase when a hydroxide or a carbonate is used as the kind of raw material to be blended compared with when an oxide is used. Further, pore volume tends to increase if calcining is not carried out, or if the calcination temperature is low, or if the sintering temperature is low or the sintering time is short.

Peak pore size tends to decrease by increasing the crushing degree of the used raw materials, especially the raw materials after calcining, to make the crushed primary particles finer. Further, peak pore size can be decreased more during sintering by introducing a reducing gas such as hydrogen or carbon monoxide rather than using an inert gas such as nitrogen.

Further, pore size unevenness can be reduced by uniformly advancing the sintering properties of the raw materials during sintering. Specifically, rather than using a tunnel continuous furnace, it is preferred to use a rotary electric furnace capable of uniformly heating the raw materials. Further, pore size unevenness can also be reduced by increasing the crushing degree of the used raw materials, especially the raw materials after calcining, to make the crushed particle size distribution sharper.

By carrying out these control methods individually or in combination, a porous ferrite core material having a desired pore volume, peak pore size, and pore size unevenness can be obtained.

Resin is filled in the resultant porous ferrite core material. Various methods may be used for the filling method. Examples thereof include a dry method, a spray-dry method using a fluidized bed, a rotary-dry method, and liquid immersion-dry method using a universal stirrer. The resin used here is as described above.

In the above-described step for filling the resin, it is preferred to fill the resin in the voids of the porous ferrite core material while mixing and stirring the porous ferrite core material and the resin to be filled under reduced pressure. By filling the resin under reduced pressure in this manner, the resin can be filled into the voids efficiently. The level of reduced pressure is preferably 10 to 700 mmHg. If the level is more than 700 mmHg, there is no effect of reduced pressure, while if the level is less than 10 mmHg, the resin solution tends to boil during the filling step, making it impossible to carry out the filling efficiently.

It is preferred to divide the above-described step for filling the resin into a plurality of steps. However, it is possible to fill the resin in one filling step, and it is not absolutely necessary to divide this step into a plurality of steps. Nevertheless, when filling a large amount of resin in one attempt, for some resins agglomeration of the particles occurs. If an agglomeration is produced, and this agglomeration is used in a developing apparatus as a carrier, the agglomeration may break apart from the stirring stress of the developing apparatus. Since the charge properties on the surface boundary of the agglomerated particles vary widely, charge variation can occur over time, which is not preferable. In such a case, by dividing up the filling step into a plurality of steps, the filling can be carried out without any excess while preventing agglomeration.

After the resin has been filled, the heated and filled resin may optionally be adhered to the core material by various

techniques. The heating may be performed using external heating or internal heating, and may use, for example, a fixed-type or flow-type electric furnace, rotary electric furnace or burner furnace. The heating may even be performed by baking using microwaves. Although the temperature depends on the resin to be filled, a temperature equal to or above the melting point or the glass transition temperature is necessary. For a thermosetting resin, a condensation-crosslinking resin and the like, by increasing the temperature to the point where sufficient curing proceeds, a resin-filled carrier which is strong against shocks can be obtained.

As described above, after the resin is filled in the porous ferrite core material, it is preferred to coat the surface with a resin. Carrier properties, and especially electrical properties such as charge properties, are often affected by the materials present on the carrier surface and the shape of the carrier surface. Therefore, by coating the surface with a suitable resin, the desired carrier properties can be adjusted with good precision. Examples of the coating method include conventionally-known methods, such as brush coating, dry method, spray-dry method using a fluidized bed, rotary-dry method and liquid immersion-dry method using a universal stirrer. To improve the coating efficiency, a method using a fluidized bed is preferable. After coating the resin, baking may be carried out by either external heating or internal heating. The baking can be carried out using, for example, a fixed-type or flow-type electric furnace, rotary electric furnace, burner furnace, or even by using microwaves. In the case of using a UV-curable resin, a UV heater is used. Although the baking temperature depends on the resin which is used, the temperature must be equal to or higher than the melting point or the glass transition point. For a thermosetting resin or a condensation-crosslinking resin, the temperature must be increased to a point where sufficient curing proceeds.

<Electrophotographic Developer According to the Present Invention>

Next, the electrophotographic developer according to the present invention will be described.

The electrophotographic developer according to the present invention is composed of the above-described resin-filled carrier for an electrophotographic developer and a toner.

Examples of the toner particles constituting the electrophotographic developer according to the present invention include crushed toner particles produced by a crushing method, and polymerized toner particles produced by a polymerizing method. In the present invention, toner particles obtained by either method can be used.

The crushed toner particles can be obtained, for example, by thoroughly mixing a binding resin, a charge control agent, and a colorant with a mixer such as a Henschel mixer, then melting and kneading with a twin screw extruder or the like, cooling, crushing, classifying, adding with additives, and then mixing with a mixer or the like.

The binding resin constituting the crushed toner particle is not especially limited, and examples thereof include polystyrene, chloropolystyrene, styrene-chlorostyrene copolymer, styrene-acrylate copolymer and styrene-methacrylate copolymer, as well as a rosin-modified maleic acid resin, epoxide resin, polyester resin and polyurethane resin. These may be used alone or by mixed together.

An arbitrary charge control agent may be used. Examples of a positively-charged toner include a nigrosin dye and a quaternary ammonium salt, and examples of a negatively-charged toner include a metal-containing monoazo dye.

As the colorant (coloring material), conventionally known dyes and pigments can be used. Examples include carbon

black, phthalocyanine blue, permanent red, chrome yellow, phthalocyanine green. In addition, additives such as a silica powdered body and titania for improving the fluidity and cohesion resistance of the toner can be added according to the toner particles.

Polymerized toner particles are produced by a conventionally known method such as suspension polymerization, emulsion polymerization, emulsion coagulation, ester extension and phase transition emulsion. The polymerization method toner particles can be obtained, for example, by mixing and stirring a colored dispersion liquid in which a colorant is dispersed in water using a surfactant, a polymerizable monomer, a surfactant and a polymerization initiator in an aqueous medium, emulsifying and dispersing the polymerizable monomer in the aqueous medium, and polymerizing while stirring and mixing. Then, the polymerized dispersion is charged with a salting-out agent, and the polymerized particles are salted out. The particles obtained by the salting-out are filtered, rinsed and dried to obtain the polymerized toner particles. Subsequently, an additive may optionally be added to the dried toner particles.

Further, during the production of the polymerized toner particles, a fixation improving agent and a charge control agent can be blended in addition to the polymerizable monomer, surfactant, polymerization initiator, and colorant, thereby allowing the various properties of the polymerized toner particles to be controlled and improved. A chain-transfer agent can also be used to improve the dispersibility of the polymerizable monomer in the aqueous medium and to adjust the molecular weight of the obtained polymer.

The polymerizable monomer used in the production of the above-described polymerized toner particles is not especially limited, and examples thereof include styrene and its derivatives, ethylenic unsaturated monoolefins such as ethylene and propylene, halogenated vinyls such as vinyl chloride, vinyl esters such as vinyl acetate, and  $\alpha$ -methylene aliphatic monocarboxylates, such as methyl acrylate, ethyl acrylate, methyl methacrylate, ethyl methacrylate, 2-ethylhexyl methacrylate, dimethylamino acrylate, and diethylamino methacrylate.

As the colorant (coloring material) used for preparing the above polymerized toner particles, conventionally known dyes and pigments are usable. Examples include carbon black, phthalocyanine blue, permanent red, chrome yellow and phthalocyanine green. The surface of colorants may be improved by using a silane coupling agent, a titanium coupling agent and the like.

As the surfactant used for the production of the above polymerized toner particle, an anionic surfactant, a cationic surfactant, an amphoteric surfactant, and a nonionic surfactant can be used.

Here, examples of anionic surfactants include sodium oleate, a fatty acid salt such as castor oil, an alkyl sulfate such as sodium lauryl sulfate, and ammonium lauryl sulfate, an alkylbenzene sulfonate such as sodium dodecylbenzene sulfonate, an alkylnaphthalene sulfonate, an alkylphosphate, a naphthalenesulfonic acid-formalin condensate, and a polyoxyethylene alkyl sulfate. Examples of nonionic surfactants include a polyoxyethylene alkyl ether, a polyoxyethylene aliphatic acid ester, a sorbitan aliphatic acid ester, a polyoxyethylene alkyl amine, glycerin, an aliphatic acid ester, and an oxyethylene-oxypropylene block polymer. Further, examples of cationic surfactants include alkylamine salts such as laurylamine acetate, and quaternary ammonium salts such as lauryltrimethylammonium chloride and stearyltrimethylammonium chloride. In addition, examples of amphoteric surfactants include an aminocarbonate and an alkylamino acid.

## 15

A surfactant like that above can be generally used in an amount within the range of 0.01 to 10% by weight of the polymerizable monomer. Since the used amount of this surfactant affects the dispersion stability of the monomer as well as the environmental dependency of the obtained polymerized toner particles, the surfactant is preferably used in an amount within the above range where the dispersion stability of the monomer is secured, and the environmental dependency of the polymerized toner particles is unlikely to be excessively affected.

For the production of the polymerized toner particles, a polymerization initiator is generally used. Examples of polymerization initiators include water-soluble polymerization initiators and oil-soluble polymerization initiators, and either of them can be used in the present invention. Examples of water-soluble polymerization initiators which can be used in the present invention include persulfate salts such as potassium persulfate and ammonium persulfate, and water-soluble peroxide compounds. Examples of oil-soluble polymerization initiator include azo compounds such as azobisisobutyronitrile, and oil-soluble peroxide compounds.

In the case where a chain-transfer agent is used in the present invention, examples of the chain-transfer agent include mercaptans such as octylmercaptan, dodecylmercaptan and tert-dodecylmercaptan, and carbon tetrabromide.

Further, in the case where the polymerized toner particles used in the present invention contain a fixation improving agent, examples thereof include a natural wax such as carnauba wax, and an olefinic wax such as polypropylene and polyethylene.

In the case where the polymerized toner particles used in the present invention contain a charge control agent, the charge control agent which is used is not especially limited. Examples include a nigrosine dye, a quaternary ammonium salt, an organic metal complex, and a metal-containing monoazo dye.

Examples of the additive used for improving the fluidity etc. of the polymerized toner particles include silica, titanium oxide, barium titanate, fluororesin microparticles and acrylic resin microparticles. These can be used alone or in combination thereof.

Further, examples of the salting-out agent used for separating the polymerized particles from the aqueous medium include metal salts such as magnesium sulfate, aluminum sulfate, barium chloride, magnesium chloride, calcium chloride, and sodium chloride.

The average particle size of the toner particles produced as above is in the range of 2 to 15  $\mu\text{m}$ , and preferably in the range of 3 to 10  $\mu\text{m}$ . Polymerized toner particles have higher uniformity than crushed toner particles. If the toner particles are less than 2  $\mu\text{m}$ , charging capability is reduced, whereby fogging and toner scattering tend to occur. If the toner particles are more than 15  $\mu\text{m}$ , this becomes a factor in deteriorating image quality.

By mixing the thus-produced carrier with a toner, an electrophotographic developer can be obtained. The mixing ratio of the carrier to the toner, namely, the toner concentration, is preferably set to be 3 to 15% by weight. If the concentration is less than 3% by weight, a desired image density is hard to obtain. If the concentration is more than 15% by weight, toner scattering and fogging tend to occur.

A developer obtained by mixing the thus-produced carrier and a toner can be used as a supply developer. In this case, the mixing ratio of the carrier and the toner may be 2 to 50 parts by weight of toner based on 1 part by weight of carrier.

The thus-prepared electrophotographic developer according to the present invention can be used in digital copying

## 16

machines, printers, FAXs, printing presses and the like, which use a development system in which electrostatic latent images formed on a latent image holder having an organic photoconductor layer are reversal-developed by the magnetic brushes of a two-component developer having the toner and the carrier while impressing a bias electric field. The present developer can also be applied in full-color machines and the like which use an alternating electric field, which is a method that superimposes an AC bias on a DC bias, when the developing bias is applied from magnetic brushes to the electrostatic latent image side.

The present invention will now be described in more detail based on the following examples. However, the present invention is in no way limited to these examples.

## Example 1

Raw materials were weighed out in a ratio of 35 mol % of MnO, 14.5 mol % of MgO, 50 mol % of  $\text{Fe}_2\text{O}_3$  and 0.5 mol % of SrO. The resultant mixture was crushed for 5 hours by a wet media mill to obtain a slurry. This slurry was dried by a spray drier to obtain spherical particles. Manganomanganic oxide was used for the MnO raw material, magnesium hydroxide was used for the MgO raw material, and strontium carbonate was used as the SrO raw material. The particles were adjusted for particle size, and then heated for 2 hours at 950° C. to carry out calcination. Subsequently, the particles were crushed for 1 hour by a wet ball mill using stainless steel beads  $\frac{1}{8}$  inch in diameter, and then crushed for a further 4 hours using stainless steel beads  $\frac{1}{16}$  inch in diameter. The particle size (crushed primary particle size) of this slurry was measured using a Microtrac. The results showed that  $D_{50}$  was 2.95  $\mu\text{m}$ . The slurry was charged with an appropriate amount of dispersant. To ensure the strength of the particles to be granulated, the slurry was also charged with 0.6% by weight of PVA (20% solution) based on solid content as a binder. The slurry was then granulated and dried by a spray drier. The resultant granules were adjusted for particle size, and then heated at 650° C. for 2 hours to remove the organic components such as the dispersant and the binder.

The resultant granules were held at a temperature of 900° C. for 1 hour in a rotary electric furnace to carry out sintering. At this stage, hydrogen gas was introduced into the furnace so that the furnace interior had a reducing atmosphere.

Then, the sintered material was crushed and further classified for particle size adjustment. Low magnetic particles were then separated off by magnetic separation to obtain a core material of porous ferrite particles. This porous ferrite core material had a pore volume of 0.129 mL/g, a peak pore size of 0.52  $\mu\text{m}$ , and pore size unevenness dv of 0.15.

Next, a condensation-crosslinking silicone resin formed from T units and D units (weight average molecular weight of about 8000) was prepared, and 100 parts by weight of the above-described porous ferrite particles and 60 parts by weight of this silicone resin in solution (since the resin solution concentration was 20%, 12 parts by weight as solid content, with a toluene diluent solvent) were mixed and stirred at 60° C. under a reduced pressure of 2.3 kPa. Then, while volatilizing the toluene, the resin permeated into the porous ferrite core material interior and was filled therein.

Once it was confirmed that the toluene had sufficiently volatilized, the stirring was continued for a further 30 minutes. After the toluene had almost completely been removed, the product was taken out of the apparatus and placed in a vessel. This vessel was then placed in a hot air heating oven, and the product was heat treated for 2 hours at 220° C.

17

Then, the product was cooled to room temperature, and the ferrite particles having resin which had been cured were removed. Particle agglomerates were broken up using a vibrating sieve with 200 M apertures. Using a magnetic separator, non-magnetic matter was removed. Then, again using the vibrating sieve, coarse particles were removed to obtain a resin-filled carrier filled with resin.

## Example 2

A resin-filled carrier was obtained in the same manner as in Example 1, except for the following changes. Used as the core material was a porous ferrite particles obtained by changing the sintering conditions to holding for 1 hour at a temperature of 950° C. in a rotary electric furnace under a reducing atmosphere obtained by introducing hydrogen gas into the furnace. This porous ferrite particles had a pore volume of 0.073 mL/g, a peak pore size of 0.42  $\mu\text{m}$ , and a pore size unevenness dv of 0.26. Further, the resin filled amount was 10 parts by weight as solid content.

## Example 3

A resin-filled carrier was obtained in the same manner as in Example 1, except for the following changes. Used as the core material was a porous ferrite particles obtained by changing the post-calcination crushing conditions to crushing for 1 hour by a wet ball mill using stainless steel beads  $\frac{1}{8}$  inch in diameter, and then crushing for a further 10 hours using stainless steel beads  $\frac{1}{16}$  inch in diameter so that the slurry particle size (crushed primary particle size) had a finer  $D_{50}$  of 1.03  $\mu\text{m}$ ; and also only changing the sintering conditions to holding for 1 hour at a temperature of 850° C. in a rotary electric furnace under a reducing atmosphere obtained by introducing hydrogen gas into the furnace. This porous ferrite particles had a pore volume of 0.152 mL/g, a peak pore size of 0.30  $\mu\text{m}$ , and a pore size unevenness dv of 0.20.

## Example 4

A resin-filled carrier was obtained in the same manner as in Example 1, except for the following changes. Used as the core material was a porous ferrite particles obtained by changing the sintering conditions to holding for 1 hour at a temperature of 900° C. in a rotary electric furnace under a reducing atmosphere obtained by introducing hydrogen gas into the furnace, and then further holding for 1 hour at a sintering temperature of 1,150° C. in the same rotary electric furnace in an inert atmosphere of nitrogen. This porous ferrite particles had a pore volume of 0.092 mL/g, a peak pore size of 0.70  $\mu\text{m}$ , and a pore size unevenness dv of 0.31. Further, the resin filled amount was 10 parts by weight as solid content.

## Example 5

A resin-filled carrier was obtained in the same manner as in Example 1, except for the following changes. Used as the core material was a porous ferrite particles obtained by changing the sintering conditions to holding for 1 hour at a temperature of 900° C. in a rotary electric furnace under a reducing atmosphere obtained by introducing hydrogen gas into the furnace, and then further holding for 1 hour at a sintering temperature of 1,170° C. in the same rotary electric furnace in an inert atmosphere of nitrogen. This porous ferrite particles had a pore volume of 0.061 mL/g, a peak pore size of 0.67  $\mu\text{m}$ , and

18

a pore size unevenness dv of 0.32. Further, the resin filled amount was 8 parts by weight as solid content.

## Example 6

5 A resin-filled carrier was obtained in the same manner as in Example 1, except for the following changes. Used as the core material was a porous ferrite particles obtained by changing the sintering conditions to holding for 1 hour at a temperature of 900° C. in a rotary electric furnace under a reducing atmosphere obtained by introducing hydrogen gas into the furnace, and then further holding for 1 hour at a sintering temperature of 1,180° C. in the same rotary electric furnace in an inert atmosphere of nitrogen. This porous ferrite particles had a pore volume of 0.055 mL/g, a peak pore size of 0.59  $\mu\text{m}$ , and a pore size unevenness dv of 0.30. Further, the resin filled amount was 6 parts by weight as solid content.

## Comparative Example 1

10 The sintering step of Example 1 was changed as follows. Specifically, the sintering was carried out by holding for 3 hours under a nitrogen gas atmosphere, at a sintering temperature of 1,100° C., in a batch electric furnace. Then, the sintered material was crushed and further classified for particle size adjustment. Low magnetic particles were then separated off by magnetic separation to obtain a core material of porous ferrite particles. This ferrite core material had a pore volume of 0.122 mL/g, a peak pore size of 1.91  $\mu\text{m}$ , and a pore size unevenness dv of 1.39. A resin-filled carrier was obtained by carrying out the subsequent resin filling step in the same manner as in Example 1.

## Comparative Example 2

15 A resin-filled carrier was obtained in the same manner as in Comparative Example 1, except that porous ferrite which was sintered by changing the sintering temperature to 1,175° C., and had a pore volume of 0.058 mL/g, a peak pore size of 0.90  $\mu\text{m}$ , and a pore size unevenness dv of 1.33, was used as the core material, and the resin filled amount was 8 parts by weight as solid content.

## Comparative Example 3

20 A resin-filled carrier was obtained in the same manner as in Comparative Example 1, except that porous ferrite which was sintered by changing the sintering temperature to 1,200° C., and had a pore volume of 0.052 mL/g, a peak pore size of 0.61  $\mu\text{m}$ , and a pore size unevenness dv of 1.25, was used as the core material, and the resin filled amount was 3 parts by weight as solid content.

## Comparative Example 4

25 A resin-filled carrier was obtained in the same manner as in Comparative Example 1, except that porous ferrite which was sintered by changing the sintering temperature to 1,210° C., and had a pore volume of 0.032 mL/g, a peak pore size of 0.60  $\mu\text{m}$ , and a pore size unevenness dv of 1.28, was used as the core material, and the resin filled amount was 3 parts by weight as solid content.

30 The pore volume, peak pore size, pore size unevenness dv, and resin filled amount of Examples 1 to 6 and Comparative Examples 1 to 4 are shown in Table 1. Further, the respective properties and evaluation results of the obtained resin-filled carriers are shown in Table 2.

TABLE 1

| Pore        | Core material pore size |                        |             | Pore size<br>unevenness<br>dv | Resin<br>filled<br>amount<br>(parts by<br>weight) |      |
|-------------|-------------------------|------------------------|-------------|-------------------------------|---------------------------------------------------|------|
|             | volume<br>(ml/g)        | Peak pore<br>size (μm) | d16<br>(μm) |                               |                                                   |      |
| Example 1   | 0.129                   | 0.52                   | 0.61        | 0.32                          | 0.15                                              | 12.0 |
| Example 2   | 0.073                   | 0.42                   | 0.86        | 0.34                          | 0.26                                              | 10.0 |
| Example 3   | 0.152                   | 0.30                   | 0.52        | 0.12                          | 0.20                                              | 12.0 |
| Example 4   | 0.092                   | 0.70                   | 1.05        | 0.42                          | 0.31                                              | 10.0 |
| Example 5   | 0.061                   | 0.67                   | 0.97        | 0.33                          | 0.32                                              | 8.0  |
| Example 6   | 0.055                   | 0.59                   | 0.91        | 0.31                          | 0.30                                              | 6.0  |
| Comparative | 0.122                   | 1.91                   | 3.38        | 1.24                          | 1.39                                              | 12.0 |
| Example 1   |                         |                        |             |                               |                                                   |      |
| Comparative | 0.058                   | 0.90                   | 2.96        | 0.31                          | 1.33                                              | 8.0  |
| Example 2   |                         |                        |             |                               |                                                   |      |
| Comparative | 0.052                   | 0.61                   | 2.61        | 0.12                          | 1.25                                              | 3.0  |
| Example 3   |                         |                        |             |                               |                                                   |      |
| Comparative | 0.032                   | 0.60                   | 2.74        | 0.18                          | 1.28                                              | 3.0  |
| Example 4   |                         |                        |             |                               |                                                   |      |

TABLE 2

| Carrier<br>electrical<br>resistance after<br>resin filling:<br>Applied voltage:<br>100 V (Ω) | Unevenness<br>among<br>particles in<br>filled resin<br>state | Carrier<br>pycrometer |                | Carrier<br>apparent<br>density<br>(g/cm³) | Carrier<br>average<br>particle<br>size<br>d50 (μm) | Carrier<br>saturated<br>magnetization<br>(Am²/kg) |      |    |
|----------------------------------------------------------------------------------------------|--------------------------------------------------------------|-----------------------|----------------|-------------------------------------------|----------------------------------------------------|---------------------------------------------------|------|----|
|                                                                                              |                                                              | Carrier<br>strength   | Toner<br>spent |                                           |                                                    |                                                   |      |    |
| Example 1                                                                                    | 5.8 × 10⁸                                                    | ◎                     | ◎              | 98.0                                      | 3.68                                               | 1.62                                              | 37.9 | 54 |
| Example 2                                                                                    | 6.2 × 10¹⁰                                                   | ○                     | ◎              | 96.2                                      | 3.93                                               | 1.65                                              | 41.0 | 62 |
| Example 3                                                                                    | 6.0 × 10⁷                                                    | ◎                     | ○              | 95.6                                      | 3.73                                               | 1.69                                              | 39.8 | 56 |
| Example 4                                                                                    | 8.0 × 10¹²                                                   | ○                     | ◎              | 95.2                                      | 4.02                                               | 1.53                                              | 38.6 | 61 |
| Example 5                                                                                    | 7.4 × 10¹²                                                   | ○                     | ◎              | 95.3                                      | 4.08                                               | 1.62                                              | 37.5 | 64 |
| Example 6                                                                                    | 5.9 × 10¹¹                                                   | ○                     | ○              | 95.0                                      | 4.21                                               | 1.87                                              | 38.1 | 66 |
| Comparative                                                                                  | 5.3 × 10⁶                                                    | X                     | X              | 92.3                                      | 3.78                                               | 1.55                                              | 37.7 | 53 |
| Example 1                                                                                    |                                                              |                       |                |                                           |                                                    |                                                   |      |    |
| Comparative                                                                                  | 1.2 × 10¹¹                                                   | Δ                     | Δ              | 90.2                                      | 4.14                                               | 1.83                                              | 38.3 | 65 |
| Example 2                                                                                    |                                                              |                       |                |                                           |                                                    |                                                   |      |    |
| Comparative                                                                                  | 3.6 × 10¹²                                                   | Δ                     | ○              | 80.2                                      | 4.78                                               | 2.00                                              | 39.5 | 68 |
| Example 3                                                                                    |                                                              |                       |                |                                           |                                                    |                                                   |      |    |
| Comparative                                                                                  | 4.5 × 10¹²                                                   | Δ                     | Δ              | 77.0                                      | 4.84                                               | 2.12                                              | 40.3 | 71 |
| Example 4                                                                                    |                                                              |                       |                |                                           |                                                    |                                                   |      |    |

It is clear from the results shown in Table 2 that the resin-filled carriers described in Examples 1 to 6 have, due to the fact that a core material which kept a suitable pore volume, peak pore size, and pore size unevenness dv was used, and as a result of the fact that the filling of the resin was carried out sufficiently but not in excess, an electrical resistance in a preferred range and a small unevenness among particles of the filled resin. Further, under observation with an SEM after a strength test, the resin-filled carriers described in Examples 1 to 6 have chipping and splitting in an acceptable range. Further, good results were also obtained in the toner spent evaluation.

In view of these results, the resin-filled carriers described in Examples 1 to 6 have realized a reduced specific gravity, while simultaneously keeping a good breakdown voltage, and exhibiting excellent mechanical strength of the carrier particles. Therefore, if these carriers were actually used in a developer, it can be easily imagined that the occurrence of charge leakage and the crushing and deterioration of the carrier particles due to the stress in an actual machine could be prevented, and that there would be no occurrence of image defects such as white spots, whereby good image quality which is stable over time could be obtained. Further, it can be

expected that these resin-filled carriers could also be preferably used as a supply developer.

On the other hand, the carrier described in Comparative Example 1 has a large peak pore size, and a large pore volume as well, so that under observation with an SEM after the strength test, a lot of chipping and splitting was observed, meaning that mechanical strength had deteriorated. Further, since the porous ferrite core material also had a large pore size unevenness, the resin filling could not be carried out uniformly, so that a part of the porous ferrite core material was greatly exposed. As a result, it can be easily inferred that resistance and breakdown voltage would both be low possibly due to the fact that there are charge leak points, and that toner spent would also be beyond the permissible range.

Since the carrier obtained in Comparative Example 2 has a large peak pore size, under observation with an SEM after the strength test, a lot of chipping and splitting was observed, meaning that mechanical strength had deteriorated. Further, since the pore size unevenness was also large, there was unevenness among the particles in a resin filled state, so that sites were formed where toner spent tended to occur, which meant that toner spent was also beyond the permissible range.

The carriers obtained in Comparative Examples 3 and 4 had a small pore volume, so that the resin filled amount was

## 21

controlled. As a result, these carriers had a high pyconometer density, which meant that a reduced specific gravity and reduced stress could not be achieved. Further, since the pore size unevenness was also large, there was unevenness among the particles in a resin filled state, so that sites were formed where toner spent tended to occur. As a result, toner spent exhibited a very large value, which was beyond the permissible range.

As described above, if the carriers obtained in Comparative Examples 1 to 4 were actually used, it can be easily imagined that the carriers would deteriorate due to the stress in an actual machine, which would result in the charge amount changing greatly, the occurrence of charge leakage and a deterioration in strength. This would allow the formation of crushed micro-particles, so that image defects, such as white spots, caused by the microparticles would tend to occur, whereby good image quality could not be stably maintained.

The resin-filled carrier for an electrophotographic developer according to the present invention has a high breakdown voltage and a high particle breaking strength, while maintaining the advantages of resin-filled carriers.

Therefore, the resin-filled carrier for an electrophotographic developer according to the present invention can be widely used in the fields of full color machines in which high quality images are demanded, as well as high-speed printers in which the reliability and durability of image sustainability are demanded.

What is claimed is:

1. A resin-filled carrier for an electrophotographic developer obtained by filling resin into voids of a porous ferrite core material, wherein the porous ferrite core material has a pore volume of 0.055 to 0.16 mL/g and a peak pore size of 0.20 to 0.7  $\mu\text{m}$ .

2. The resin-filled carrier for an electrophotographic developer according to claim 1, wherein in a pore size distribution of the porous ferrite core material, pore size unevenness  $dv$  represented by the following formula (1) is 1.0 or less,

$$dv = |d_{84} - d_{16}|/2 \quad (1)$$

wherein  $d_{16}$  is a pore size calculated from the applied pressure on mercury when the mercury pressure penetra-

## 22

tration reaches 16%, where the total pressure penetration in the high pressure region is 100%; and  $d_{84}$  is a pore size calculated from the applied pressure on mercury when the mercury pressure penetration reaches 84%, in which the total pressure penetration in the high pressure region is 100%.

3. The resin-filled carrier for an electrophotographic developer according to claim 1, wherein the resin is filled in the porous ferrite core material in an amount of 6 to 30 parts by weight based on 100 parts by weight of the porous ferrite core material.

4. The resin-filled carrier for an electrophotographic developer according to claim 1, having an average particle size of 20 to 60  $\mu\text{m}$ .

5. The resin-filled carrier for an electrophotographic developer according to claim 1, having a saturated magnetization of 30 to 80  $\mu\text{m}^2/\text{kg}$ .

6. The resin-filled carrier for an electrophotographic developer according to claim 1, having a pyconometer density of 2.5 to 4.5  $\text{g}/\text{cm}^3$ .

7. The resin-filled carrier for an electrophotographic developer according to claim 1, having an apparent density of 1.0 to 2.5  $\text{g}/\text{cm}^3$ .

8. An electrophotographic developer comprising the resin-filled carrier according to claim 1 and a toner.

9. A supply developer comprising the electrophotographic developer according to claim 8.

10. An electrophotographic developer comprising the resin-filled carrier according to claim 2 and a toner.

11. An electrophotographic developer comprising the resin-filled carrier according to claim 3 and a toner.

12. An electrophotographic developer comprising the resin-filled carrier according to claim 4 and a toner.

13. An electrophotographic developer comprising the resin-filled carrier according to claim 5 and a toner.

14. An electrophotographic developer comprising the resin-filled carrier according to claim 6 and a toner.

15. An electrophotographic developer comprising the resin-filled carrier according to claim 7 and a toner.

\* \* \* \* \*